# EUROPEAN PATENT SPECIFICATION

(11) **EP 0 024 277 B1**
(45) Date of publication and mention of the grant of the patent: **26.01.1983**
(21) Application number: 79301690.8
(22) Date of filing: 17.08.1979
(51) Int. Cl.: D01F 9/22, D01F 9/20, D01F 9/14

(54) **Process for the manufacture of graphite fibres**
Verfahren zur Herstellung von Graphitfasern
Procédé de fabrication de fibres graphitiques

(43) Date of publication of application: 04.03.1981
(73) Proprietor: TORAY INDUSTRIES, INC., Tokyo 103 (JP)
(72) Inventor: Yamamoto, Ryuichi, Iyo-Gun Ehime-Ken (JP); Watanabe, Shizuo, Iyo-Gun Ehime-Ken (JP)
(74) Representative: Ellis, John Clifford H.

## Description

Graphite fibres are generally different from carbon fibres in respect of carbon content (purity), structure and physical characteristics. Graphite fibres are preferable to carbon fibres for use in sports equipment such as fishing rods and golf club shafts which require high modulus, for use in electric components such as heaters which require high purity and low resistivity, and for use in the aerospace industry, where parts for aircraft, rockets etc., may have to have high oxidation resistivity and be made to high precision. However, graphite fibres cost much more than carbon fibres and this high cost is largely a result of difficulties in manufacturing processability and productivity. An inert atmosphere is required for production of graphite fibres, and a higher temperature is used than for carbon fibres.

Efforts have been made to increase productivity in manufacturing graphite fibres. For example, it has been proposed to increase the temperature gradient and to shorten the time in graphitizing furnace. However, this produces increased amounts of fuzz on the surface of the graphite fibres and occasional breakage of the fibre strands.

Also, these modifications tend to reduce the tensile strength of the fibres. Further, since the temperature of the inert atmosphere must be higher than that used for manufacturing carbon fibres the wear on the graphitizing furnace, particularly on its heating pipes, is considerably greater. As a result of such wear due to exceedingly high temperatures, deviations from the desired temperature profile tend to increase and the furnace tube must be changed frequently. This seriously interferes with production and processability, and also consumes large amounts of energy, labour and materials.

In FR-A-2178193 a fibre spun from a type of carbonaceous pitch, which is oxidised at 250°C to 400°C, is converted to a carbon fibre by heating in an inert atmosphere to a temperature of at least 1000°C and this carbon fibre may then be converted to a graphite fibre by heating in an inert atmosphere to a temperature of at least 2500°C.

According to FR-A-2006543, a process for the manufacture of carbon and graphite fibres comprises continuously passing a number of tapes or sheets of fibres of polyacrylonitrile or a copolymer thereof (being at least 10⁵ fibres) through a preoxidation furnace, a carbonising furnace at a temperature of 500-1200⁰C in an inert atmosphere and a graphitising furnace at a temperature of 1500°C-3000°C in an inert atmosphere.

According to the present invention, we start from a precursor fibre derived from polyacrylonitrile and we pass this fibre in an inert atmosphere through two separately controllable heating zones, of which the temperature and the average heating rate is within or above certain limits. Specifically the temperature at the hottest point in the first heating zone is to be within the range 1500-2100°C, with an average rate of heating in this zone being from 300°C/min to 2000°C/min, and the temperature at the hottest point in the second heating zone is to be at least 2100°C with an average rate of heating in this zone of from 2000°C/min to 10,000°C/min.

By use of the present invention it is possible to obtain a stable method of manufacturing high grade and high quality graphite fibres, particularly graphite fibres which have a minimum of surface fuzz. The process may use a shorter heating zone than is usual in conventional processes. Additionally, it is possible to provide a manufacturing process in which the life of parts is lengthened, and their replacement is easier, thereby saving energy, materials and labour.

The term "graphite fibre" as used herein is intended to mean a fibre which is obtained by heating a graphitizable precursor fibre in an inert atmosphere at a temperature of 2100°C or more and which fibre contains about 95% or more by weight of carbon. The term "graphitizable precursor fibre" or "precursor fibre" is intended to mean a fibre which has sufficient structural integrity to maintain its fibrous character and which can be converted to a graphite fibre when heated in an inert atmosphere at a temperature of 2100°C or more. A typical example of a precursor fibre is an oxidized fibre obtained by heating a polyacrylonitrile fibre in an oxidizing atmosphere at a temperature of about 200°C to 400°C. Another typical example is a carbon fibre obtained by heating the said oxidized fibre in an inert atmosphere at a temperature between 400°C and 1500°C. When using the process of the present invention it is preferable to use a precursor fibre obtained from an acrylic fibre comprising about 95 mol % minimum of acrylonitrile (AN) and up to about 5 mol % of one or more ethylene-type vinyl compounds which are copolymerizable with acrylonitrile.

The maximum temperature in the first heating zone is preferably in the range of 1700°C to 1900°C. The second heating zone preferably has a maximum temperature in the range of 2100°C to 3500°C, more preferably in the range of 2300°C to 2700°C.

It has been discovered that if the front and rear heating zones are operated at heating temperatures outside the ranges from 1500°C to 2100°C and 2100°C to 3500°C, respectively, it is difficult to obtain high quality graphite fibre. The quality of the fibre produced is influenced by such things as the type of precursor fibre, whether it was pretreated or not, and the temperature profile of the heating zone; in some instances it is especially sensitive to the maximum temperature of the first heating zone and is reduced if this exceeds about 2100°C. In particular, the fibres tend to develop excessive surface fuzz and tend to break easily.

The rate of heating of the precursor fibre as it passes through the heating zones is within the range of 300°C/min to 2000°C/min in the first heating zone, more preferably within the range of 500°C/min to 1500°C/min, and within the range of 2000°C/min to 10,000°C/min in the second heating zone.

The treatment time of the precursor fibres in the first heating zone, which is defined as the time during which the fibres are in the zone at a temperature above 1000°C is preferably within the range of 10 seconds to 10 minutes, more preferably 30 seconds to 3 minutes.

An embodiment of the present invention will now be described by way of example with reference to the drawings, in which:
Fig. 1 is a view in longitudinal section of graphitizing apparatus for carrying out the process of this invention;
Figs. 2 and 3 respectively show typical examples of temperature profiles in the furnace tubes used in the respective heating zones.

Referring to Fig. 1, the separate first and second heating zones (furnaces) have respectively furnace tubes (2, 3) to which heat is applied in a conventional way. The furnace tubes (2, 3) are surrounded with insulation (4, 5). An inert gas such as nitrogen is supplied to the furnaces (I, II) through pipes (6), and the gas is removed from the furnaces by pipes (7). At each end of each furnace there are furnace seals (8), supplied with inert gas through supply pipes (9).

As shown in Fig. 1, the precursor fibre (1) is first conducted through the seal (8) into the furnace tube (2) of the furnace (1) which provides the first heating zone. The temperature profile inside this furnace tube (2) is controlled, to produce a profile as shown in Fig. 2. This is done by locally controlling the heat input at selected spots along the tube (2), in a conventional way. When the precursor fibre is a carbon fibre, it is treated in this furnace until its weight is reduced to about 93% to 95% of its previous weight, and then it is conducted into the furnace tube (3) of the furnace (II) which provides the second heating zone. There the fibre is heated again, and is converted into a graphite fibre. Fig. 3 shows a typical temperature profile of the furnace tube (3) of the second heating zone, the maximum temperature of which is set at about 2500°C in this case.

By use of the present invention, a more efficient and therefore more profitable process for the manufacture of graphite fibres is possible. These advantages can be realised for the following reasons:
(a) The heating zone is divided into two independently controlled zones, giving increased flexibility with the rate of heating the fibre. There is also better control of the temperature profile within the furnace;
(b) The weight loss of the precursor fibre during initial heating up to 1500°C is usually large. It has been found that the use of a high rate of heating in the stage up to 1 500°C tends to damage the precursor fibre. In the conventional, single heating zone system, the overall rate of heating must be so low that it restricts overall productivity. By use of the present, double heating zone system, it is possible to select optimum rates of heating for the first and second heating zones independently of each other. This allows manufacture of high quality graphite fibres with increased productivity;
(c) With the process of the present invention, it is possible to reduce the overall length of the heating zone by dividing it, and the maintenance and custody of the furnace can thereby be made easier. The life of a furnace tube in the second furnace is much shorter than that of one in the first furnace, because of the higher temperature at which it operates. However, clearly the tube in the first furnace need not be replaced merely because the tube in the second furnace has to be, and also the tube in the second furnace, being relatively short compared with the tube in a single-heating zone furnace, is easier to handle. Thus, costs of time, labour, and materials can be reduced. Surprisingly the energy consumption can also be reduced. This is because it has been found possible to string up the fibres without lowering the temperature of the furnace.

### Examples

Carbon fibres were produced from acrylic fibres and carbonized in an inert atmosphere, the maximum temperature of which was 1100°C. They were taken from creels and heated to produce graphite fibres using separate furnaces as shown in Fig. 1. The conditions were varied, there being 3 conditions within the scope of the invention (Examples 1-3) and four conditions outside the scope of the invention (Comparative Examples 1-4). The conditions are shown in Table 1.

The resulting data are shown in Table 2. Moreover, the usual temperatures, the periods of time between changes of furnace tubes and the number of days required to change them, with respect to both first and second furnaces, are shown in Table 3. Some of the properties of the fibres made in these examples are shown in Table 2.

Table 3 gives an indication of the lifetime of the furnace tubes, at different operating temperatures, and the time taken to change them.

## Claims

1. A process for the manufacture of graphite fibre by graphitizing precursor fibre derived from a polyacrylonitrile fibre characterised in that the precursor fibre or fibres pass successively through separately controllable first and second heating zones, both containing an inert atmosphere, the temperature at the hottest point in the said first heating zone being in the range of 1500°C to 2100°C, the average rate of heating of fibre in the first heating zone being in the range of from 300°C/min to 2000°C/min, the temperature at the hottest part in the said second heating zone being at least 2100°C and the average rate of heating of fibre in the second heating zone being in the range of from 2000°C/min to 10,000°C/min.

2. A process according to claim 1 in which the two heating zones are constituted by separate furnace tubes separately heated and furnished with inert atmosphere.

3. A process according to claim 1 or claim 2 in which the said temperature at the hottest point in the first heating zone is in the range of from 1700°C to 1900°C.

4. A process according to any one of claims 1 to 3 in which the said temperature at the hottest point in the second heating zone is in the range of 2100°C to 3500°C.

5. A process according to claim 4 in which the said temperature at the hottest point in the second heating zone is in the range of from 2300°C to 2700°C.

6. A process according to any one of the preceding claims in which the precursor fibre is a carbon fibre obtained from an acrylic fibre comprising at least 95 mol % of acrylonitrile and up to 5 mol % of one or more ethylene-type vinyl compounds copolymerizable with acrylonitrile by heating and oxidizing the said acrylic fibre in an oxidizing atmosphere at a temperature in the range of 200°C to 400°C, and then heating the oxidized fibre so formed in an inert atmosphere at a temperature of from 400°C to 1500°C.

7. A process according to any one of claims 1 to 5 in which the precursor fibre is an oxidized fibre obtained from an acrylic fibre comprising at least 95 mol % of acrylonitrile and up to 5 mol % of one or more ethylene-type vinyl compounds copolymerizable with acrylonitrile, by heating and oxidizing the said acrylic fibre in an oxidizing atmosphere at a temperature of from 200°C to 400°C.

## Patentansprüche

1. Verfahren zur Herstellung von Graphitfaser durch Graphitieren einer von einer Polyacrylnitrilfaser abgeleiteten Vorstufenfaser, dadurch gekennzeichnet, daß die Vorstufenfaser oder -fasern nacheinander durch eine getrennt steuerbare erste und zweite Heizzone hindurchtreten, deren beide eine Inertatmosphäre enthalten, wobei die Temperatur am heißesten Punkt der ersten Heizzone im Bereich von 1500°C bis 2100°C liegt, die mittlere Aufheizgeschwindigkeit der Faser in der ersten Heizzone im Bereich von 300°C/min bis 2000°C/min liegt, die Temperatur im heißesten Bereich der zweiten Heizzone mindestens 2100°C beträgt und die mittlere Aufheizgeschwindigkeit der Faser in der zweiten Heizzone im Bereich von 2000°C/min bis 10000°C/min liegt.

2. Verfahren nach Anspruch 1, bei dem die beiden Heizzonen durch getrennte Ofenrohre gebildet sind, die getrennt geheizt und mit Inertatmosphäre beliefert sind.

3. Verfahren nach Anspruch 1 oder 2, bei dem die Temperatur am heißesten Punkt der ersten Heizzone im Bereich von 1700°C bis 1900°C liegt.

4. Verfahren nach einem der Ansprüche 1 bis 3, bei dem die Temperatur am heißesten Punkt der zweiten Heizzone im Bereich von 2100°C bis 3500°C liegt.

5. Verfahren nach Anspruch 4, bei dem die Temperatur am heißesten Punkt der zweiten Heizzone im Bereich von 2300°C bis 2700°C liegt.

6. Verfahren nach einen der vorhergehenden Ansprüche, bei dem die Vorstufenfaser eine Kohlenstoffaser ist, die aus einer mindestens 95 mol % Acrylnitril und bis zu 5 mol % einer oder mehrerer mit Acrylnitril kopolymerisierbarer äthylenartiger Vinylverbindungen enthaltenden Acrylfaser durch Erhitzen und Oxidieren der Acrylfaser in einer oxidierenden Atmosphäre bei einer Temperatur im Bereich von 200°C bis 400°C und sodann durch Erhitzen der solchermaßen gebildeten oxidierten Faser in einer Inertatmosphäre bei einer Temperatur von 400°C bis 1500°C erhalten wird.

7. Verfahren nach einem der Ansprüche 1 bis 5, bei dem die Vorstufenfaser eine oxidierte Faser ist, die aus einer mindestens 95 mol % Acrylnitril und bis zu 5 mol % einer oder mehrerer mit Acrylnitril kopolymerisierbarer äthylenartiger Vinylverbindungen enthaltenden Acrylfaser durch Erhitzen und Oxidieren der Acrylfaser in einer oxidierenden Atmosphäre bei einer Temperatur von 200°C bis 400°C erhalten wird.

## Revendications

1. Procédé de fabrication de fibres de graphite par graphitisation d'une fibre précurseur dérivée d'une fibre polyacrylonitrile, caractérisé en ce que la fibre précurseur ou fibres passent successivement à travers des première et seconde zones de chauffage contrôlables de façon séparée, contenant toutes les deux une atmosphère inerte, la température au point le plus chaud dans ladite première zone de chauffage étant dans la gamme de 1500°C à 2100°£, la vitesse moyenne de chauffage des fibres dans la première zone de chauffage étant dans la gamme de 300°C/mn à 2000°C/mn, la température à la partie la plus chaude dans la seconde zone de chauffage étant d'au moins 2100°C et la vitesse moyenne de chauffage des fibres dans la seconde zone de chauffage étant dans la gamme de 2000°C/mn à 10 000°C/mn.

2. Procédé selon la revendication 1, dans lequel les deux zones de chauffage sont constituées par des tubes de four séparés chauffés de façon séparée et fournis en atmosphère inerte.

3. Procédé selon la revendication 1 ou 2, dans lequel la température précitée au point le plus chaud dans la première zone de chauffage est dans la gamme de 1700°C à 1900°C.

4. Procédé selon l'une des revendications 1 à 3, dans lequel la température précitée au point le plus chaud dans la seconde zone de chauffage est dans la gamme de 2100°C à 3500°C.

5. Procédé selon la revendication 4, dans lequel la température précitée au point le plus chaud dans la seconde zone est dans la gamme de 2300°C à 2700°C.

6. Procédé selon l'une des revendications précédentes, dans lequel la fibre précurseur est une fibre de carbone obtenue à partir d'une fibre acrylique comprenant au moins 95% en moles d'acrylonitrile et jusqu'à 5% en moles d'un ou plus de composés du type vinylique-éthylène copoly- mérisables avec l'acrylonitrile en chauffant et oxydant ladite fibre acrylique dans une atmosphère oxydante à une température dans la gamme de 200°C à 400°C, et en chauffant ensuite la fibre oxydée ainsi formée dans une atmosphère inerte à une température de 400°C à 1 500°C.

7. Procédé selon l'une des revendications 1 à 5, dans lequel la fibre précurseur est une fibre oxydée obtenue à partir d'une fibre acrylique comprenant au moins 95% en moles d'acrylonitrile et jusqu'à 5% en moles d'un ou plus de composés de type vinylique-éthylène copolymérizables avec l'acrylonitrile, en chauffant et oxydant ladite fibre acrylique dans une atmosphère oxydante à une température de 200°C à 400°C.
